

1

2,840,517

## NICKEL-IRON-ZINC ALLOY ELECTROPLATING

Charles L. Faust and William H. Safranek, Columbus, Ohio, assignors, by mesne assignments, to Rockwell Spring and Axle Company, Coraopolis, Pa., a corporation of Pennsylvania

No Drawing. Application July 10, 1957  
Serial No. 670,871

8 Claims. (Cl. 204—43)

This invention relates to nickel electroplating, particularly to a method and plating bath for obtaining a leveling, ductile, and bright nickel alloy electroplate. This application is a continuation-in-part of copending U. S. patent application Serial No. 368,903, filed July 20, 1953, now abandoned.

Nickel electroplates are conventionally employed as corrosion-resistant coatings for steel and as base plates upon which more attractive and resistant chromium electroplates are deposited. Commonly, a "flash" coat or an extremely thin coating of copper is applied to the steel article to improve the adherence of the nickel. A thicker nickel plate is then applied, followed by the chromium deposit. In the past, in order to obtain a bright and smooth-finish (level) electroplate, whether the electroplate consists of a plate of nickel alone or of a plate of nickel followed by a plate of chromium, it has been necessary to grind and polish the steel base material or the nickel electroplate, or both, to a relatively level and bright surface. This is so because scratches, depressions, and imperfections on the surface of the steel or nickel are transferred to the surface of the finished product.

Other requirements of nickel electroplating are the attainment of plates that possess a substantially even thickness and that are ductile. In electroplating articles of complex shapes, areas of the cathode nearest the anode receive a thicker electroplate and areas away from the anode receive a thinner electroplate than the average thickness of the deposit. This is caused by the fact that the areas nearest the anode have a relatively high current density while the areas farthest from the anode have a relatively low current density. Although these conditions exist in all nickel plating operations, the variations are different in different baths. The intensity of the condition in a given bath is referred to in terms of the "throwing power" of the bath. A nickel plating bath with good throwing power provides an electroplate of more even thickness than one with poor throwing power. Throwing power is, therefore, an important consideration in any nickel plating process. Ordinarily, acid nickel plating baths possess good throwing power, but many brighteners are known to reduce the throwing power of the bath.

2

Nickel plates, and metallic plates in general, have a tendency to be in a stressed condition, resulting in cracks and unsatisfactory noncontinuous coatings. An ideal nickel plate is ductile or unstressed as well as bright and level.

There has been much research and activity directed toward providing a ductile, level, and bright nickel electroplate that would reduce or eliminate the necessity of mechanically securing a bright and level nickel electrodeposit on a steel base material. Although some success has been obtained by adding organic brightening agents to acid nickel baths, the known practices have resulted in electroplates which lack at least one of the essential properties of ductility, leveling, and brightness. For example, many known plating baths result in bright and ductile plates but are unsatisfactory from the standpoint of leveling. Also, many brighteners adversely affect the plating conditions, particularly the throwing power.

The electroplating bath and process of the present invention have been found to be far superior to those of prior art practices in securing a ductile, level, and bright nickel electroplate and in providing good throwing power. The planeness or levelness of a metal surface may be measured by an instrument called a profilometer. This instrument provides an average reading of surface deviations in terms of root mean square (R. M. S.) microinches. Plating with nickel using prior art, bright nickel plating methods on polished steel plates with R. M. S. profilometer readings of 20 microinches, results in nickel plates with R. M. S. profilometer readings of about 19 microinches. A desired bright, ductile plate would have a reading of 9 or less R. M. S. microinches. Nickel and nickel alloy plates deposited in accordance with the present invention are ductile, have bright to brilliant mirrorlike finishes, and provide leveling to 6 microinches R. M. S. or less when applied to basis metal having a surface roughness of up to 20 R. M. S. microinches.

It is, therefore, a primary object of the present invention to provide a method and plating bath for obtaining a superior bright, ductile, and level nickel or nickel alloy electroplate.

It is also an object of the present invention to provide a nickel electroplating bath and process that reduce the necessity of buffing and polishing steel articles before electroplating in order to obtain adequate leveling.

Other objects and advantageous features will be obvious from the following specifications.

In general, the present invention relates to a process of electroplating and an acid nickel electroplating bath in conjunction therewith wherein the bath contains a combination of brightening and leveling ingredients within critical concentration limitations that give level, ductile, and bright nickel plates while retaining good throwing power. The materials added to the bath are disulfonated benzopyrone, zinc and iron. Operable ranges of bath ingredients are: nickel 17 to 233 g./l.; a disulfonated benzopyrone in an amount equivalent to from 1 to 10 g./l.

of coumarin disulfonic acid; zinc in amounts ranging from 0.03 to 1.25 g./l.; and iron within the range of from 0.3 to 5.6 g./l. Optimum results are obtained by confining the plating bath to within a range of from 34 to 120 g./l. of nickel, a disulfonated benzopyrone in an amount equivalent to from 1 to 10 g./l. of coumarin disulfonic acid, 0.03 to 0.20 grams per liter of zinc ions, and 0.5 to 3.0 g./l. of iron ions.

Nickel salts predominate in the plating bath. The bath should contain the usual incidental ingredients necessary to improve the efficiency of the plating operation, such as a buffer compound and a wetting agent. An electric current is passed through the baths from anode to cathode, while the bath is agitated and heated, to effect the most satisfactory results. Minor impurities may be present without materially affecting the resulting nickel plate. Nickel salts may be provided in the bath to provide the required range of nickel. Any suitable soluble nickel salts that will not interfere with plating conditions may be used in the bath. Most suitable salts are nickel fluoroborates, nickel chloride, nickel sulfamate, and nickel sulfate. Any or all of these salts may be used in the same bath, but preferably, for ease of control, better efficiency and results, the preferred baths are those containing a chloride salt, fluoroborate salt, or a mixture of chloride and sulfate salts. The nickel chloride salt used is preferably hydrated nickel chloride ( $\text{NiCl}_2 \cdot 6\text{H}_2\text{O}$ ). However,  $\text{NiCl}_2$  can likewise be used. The nickel fluoroborate added to the bath is generally obtainable in the form of a concentrated solution containing from 40 to 45 percent nickel fluoroborate,  $\text{Ni}(\text{BF}_4)_2$ . The nickel sulfate used is generally  $\text{NiSO}_4 \cdot 6\text{H}_2\text{O}$ .

Nickel within the ranges indicated can be obtained by providing a bath containing 75 to 1000 grams of nickel sulfate ( $\text{NiSO}_4 \cdot 6\text{H}_2\text{O}$ ) and from 25 to 60 g./l. of nickel chloride ( $\text{NiCl}_2 \cdot 6\text{H}_2\text{O}$ ), the preferred ranges being from 150 to 480 g./l. of the nickel sulfate and from 30 to 60 g./l. of the nickel chloride.

The iron and zinc are codeposited with the nickel, resulting in a nickel-rich plate having better protective properties, brightness, ductility and leveling properties than commercially pure nickel plates. The total of the zinc and iron in the plate itself may vary from as little as 0.01 percent up to about 40 percent, but preferably the total of these alloying metals is kept below 20 percent.

The metal brighteners may be added to the bath in the form of any ionizing salts, such as the chlorides, sulfates, or fluoroborates. It is not necessary that the salt correspond with the nickel salt addition, i. e., iron or zinc chloride may be added to nickel sulfate baths.

The disulfonated benzopyrone compound used is selected from the group consisting of disulfonated 1,2-benzopyrone (coumarin), 2,1-benzopyrone (isocoumarin) and 1,4-benzopyrone (chromone). The structural formulas of these compounds before sulfonation are as follows:



When these compounds are sulfonated, the acid radicals ( $\text{SO}_3\text{H}$ ) take various positions on a ring, depending on the nature of the compound and the position of the directing groups. In the case of coumarin, the radicals will be at the 6 and 3 positions. The sulfonation of isocoumarin likely occurs at the 6th and 7th or 7th and 8th positions. When chromone is sulfonated, addition probably occurs

at the 6th position and one of the 2nd, 3rd, or 8th positions.

It is also possible to use salts of such acids, the substitution products thereof, and crude-mix sulfonation products, as well as the disulfonic acids themselves. These materials are to be included in the term "disulfonated benzopyrone" as used herein. Examples of suitable compounds are the sodium and nickel salts of coumarin disulfonic acid; sodium and nickel salts of chromone disulfonic acid; sulfonated derivatives of benzopyrones and substitution products thereof; as the acid or salt of 3-methyl coumarin; 4,8 dimethyl coumarin; 6 chlorocoumarin; 3 acetylcoumarin; and 7 hydroxy coumarin. It will also be apparent that other alkyl, halo, and hydroxy derivatives of disulfonated coumarin, chromone, isochromone, etc., can be employed. These sulfonated benzopyrone compounds can be used singly or mixed together.

The disulfonated products of benzopyrone may be added to the baths of the present invention in any convenient form. For example, the addition may be made in the form of the sodium salt of coumarin disulfonic acid, the nickel salt of coumarin disulfonic acid, or it may be the reaction product of coumarin and fuming sulfuric acid.

The preferred addition is the nickel salt of coumarin disulfonic acid. In preparing such compound or reaction product, some nickel salt of coumarin monosulfonic acid will usually be present. This is because it is difficult to obtain a complete reaction in attaining the disulfonic product. It is not necessary, however, to separate the monoacid from the diacid, as the plating bath will tolerate a considerable portion of the monoacid without deleterious effects to the plating or resulting nickel alloy plate. Although the presence of the monoacid is not harmful in quantities equal to that of the diacid, an excess of monoacid is undesirable. It is, therefore, preferable that the sulfonated portion of the coumarin sulfonic acid product contain about 50 percent or more of the diacid. The preferred range of the product may be defined as from 2 to 20 g./l. of a coumarin sulfonic acid product, the sulfonated portion of which contains approximately 50 percent or more of the disulfonic acid.

Suitable sodium salts of coumarin sulfonic acid products can be readily prepared in the following manner:

100 grams of coumarin are added to 500 grams of fuming sulfuric acid (20 to 30 percent excess  $\text{SO}_3$ ) while stirring the mixture which is heated to between 96 and 98° C. After reacting for two hours, the hot mixture is cooled to 25° C. This product is capable of being used directly in the plating bath but neutralizing agents may be added to provide a proper pH. To make the sodium salt, the product is cooled to 5° C., and then slowly added to 800 milliliters of a saturated sodium chloride solution, cooled to between 0 and 5° C. After letting the mixture stand over night, the precipitate is removed by filtration, washed with saturated sodium chloride solution, purified by recrystallizing twice in hot water, and allowed to dry over night in an oven at 100° C.

To prepare the nickel salts, the reaction product of coumarin and fuming sulfuric acid is reacted with nickel carbonate instead of sodium chloride.

The active metals and sulfonated benzopyrone product can be conveniently added to the bath together; for example, an easy way to make additions of zinc and coumarin disulfonic acid at the same time is to add to the bath a solution prepared by reacting zinc oxide with the acid sulfonation product of coumarin. The ratio of zinc to coumarin sulfonic acid can be adjusted to any desired value. The ratio of 1 to 10 is convenient for formulating a new bath and for replenishing materials consumed while the bath is being operated. Much of the excess sulfuric acid is neutralized when zinc is added to the acid sulfonation product of coumarin when preparing a solution with one part of zinc and two parts of coumarin sulfonic acid. The remaining excess sulfuric acid can be

neutralized easily with nickel carbonate, nickel hydroxide, or equivalent.

Additions of any one of the brightening and leveling materials of the present invention to the acid nickel electroplating baths may effect an improvement in the resulting plating. This improvement may be in the form of improved leveling, range of brightness of the nickel plate, and ductility of the plate; but unless all three of the additions are made within the above-recited critical ranges, the plating will fail to be improved in at least one of the three categories (brightness, leveling, or ductility). Also, certain of these additions effect significantly better plating conditions in the form of throwing power of the plating bath.

Table 1 shows the effects of additions of one or more of the additives, coumarin disulfonic acid, zinc, and iron within the critical ranges contemplated by the present invention to acid nickel baths.

It is apparent from Table 1 that the acid nickel baths without additions possess no detectable leveling power and do not produce bright electroplates and that the addition of coumarin disulfonic acid alone has no detectable effect on leveling or brightness. However, the acid nickel baths with or without the addition of coumarin disulfonic acid alone have high throwing power properties and result in ductile plates. The addition of Zn alone destroys throwing power and ductility but effects a slight improvement in leveling and brightness. The addition of iron alone reduces throwing power and ductility while offering no improvements in leveling or brightness. The addition of both coumarin disulfonic acid and zinc improves leveling and brightness to some extent but reduces throwing power and ductility. The addition of both coumarin sulfonic acid and iron effects a broad range of brightness and does not adversely change the ductility or throwing power but does not provide a bath with adequate leveling. The bath containing all three of the additions of the present invention provides the best plating conditions available.

A buffer is usually added to the acid nickel plating bath to prevent sudden changes in the pH which could adversely affect the results. Buffers customarily used in the art can be added to the bath.

TABLE 1

| Ingredients, grams per liter |     |     | Leveling  | Bright range | Throwing power | Ductility |
|------------------------------|-----|-----|-----------|--------------|----------------|-----------|
| Coumarin disulfonic acid     | Zn  | Fe  |           |              |                |           |
| 0                            | 0   | 0   | None      | None         | Good           | Excellent |
| 2.5                          | 0   | 0   | do        | do           | do             | do        |
| 0                            | 0.2 | 0   | Fair      | Very narrow  | Poor           | Poor      |
| 0                            | 0   | 0.5 | None      | None         | Fair           | Do.       |
| 2.5                          | 0.2 | 0   | Excellent | Intermediate | do             | Good      |
| 2.5                          | 0   | 2.5 | Poor      | Broad        | Good           | Excellent |
| 2.5                          | 0.1 | 2.5 | Good      | do           | do             | do        |

None= no detectable brightness range or leveling effect.

Fair=some leveling effect but not significant; adequate throwing power but not so good as in baths without additions.

Excellent=significantly improved leveling; best ductility attainable.

Good=satisfactory throwing power or ductility but not the best ductility attainable.

Poor=unsatisfactory and commercially nonacceptable leveling, throwing power, or ductility.

disclosed herein in amounts to properly effect the buffering action. It has been found best to employ boric acid. From a practical standpoint, the amount of buffer generally may be from 10 to 60 g./l., although best results in control, economy, and plate conditions are obtained with concentrations of from 30 to 45 g./l.

A wetting agent is desirable to prevent pitting of the plates and is generally used in the baths of this invention.

Agents previously known to prevent pitting in nickel plates are satisfactory. It will be understood, however, that such agents must not adversely affect the baths, operating conditions and resulting electroplates. An example of a suitable wetting agent is sodium lauryl sulfate. Only a minor amount need be added to the bath to prevent pitting, and large amounts are unnecessary and wasteful. Generally, from 0.1 to 1.0 g./l. of wetting agent can be present in the bath, although from 0.2 to 0.5 g./l. is best for preventing pitting of the surfaces.

The pH of the bath is adjusted by adding to the bath a suitable acid, such as hydrochloric or sulfuric acid, or a suitable alkali, such as nickel carbonate, nickel hydroxide, or zinc oxide. The pH of the bath should always be on the acid side and preferably should not exceed about 5 for any appreciable period of time. It should never be below about 1.9 or the bath would be thrown out of balance, and the composition, levelness, and brightness of the plate would be adversely altered on continued operation. It has been found that the best bath stability and resulting plate conditions are accomplished by maintaining the pH of the bath at from 2.5 to 4.5.

The bath should always be agitated during plating in order to consistently obtain leveling plates having a bright mirrorlike appearance.

Soluble metal anodes, such as anodes of nickel, may be used. Alloy anodes may include nickel alloys containing iron and zinc which substantially replenish the bath. Current densities for the anodes should be sufficient to provide the correct dissolution, and, for most purposes, can range from 5 to 60 amperes per square foot. It is preferred to maintain the anode current density in the range of from 20 to 40 amperes per square foot in order to obtain the best results from a commercial standpoint.

Operating cathode current densities from 20 to 100 or more amperes per square foot can be used in the present method although from a practical and commercial standpoint it has been found best to employ current densities in the range of from 30 to 60 amperes per square foot.

The plating should be carried on for at least about 5 minutes. For better leveling effect, at least 15 minutes' operation is required. The plating can continue for as long as needed, although for economy and entirely satisfactory results, plating times are not generally continued beyond 60 minutes. The temperature of the plating baths must be maintained at from 80 to 180° F. The preferred temperature range is from 125 to 145° F.

The following specific examples illustrate the plating baths of the present invention, but do not restrict the present invention to the exact compositions and conditions set forth.

Table 2 shows five nickel plating baths containing sulfonated coumarin product, iron, and zinc as the brightening and leveling agents. The sulfonated coumarin was produced by sulfonating one part coumarin with five parts of 20 percent oleum (a solution of  $H_2SO_4$  and about 20 percent, by weight  $SO_3$ ). The resulting reaction product that was used as the recited addition had a coumarin disulfonic acid content of approximately 15 percent. The coumarin monosulfonic acid content of the reactive product was also about 15 percent. The wetting agent solution "XXXD" was a solution of sodium lauryl sulfate made by The Harshaw Chemical Company. All of the baths produced ductile mirror-bright nickel plates on polished steel sections.

Table 3 sets forth four examples of nickel plating baths containing nickel coumarin disulfonate, iron, and zinc as the brightening and leveling agents. The sulfonated portion of the sulfonated coumarin reaction product employed contained about 50 percent of the disulfonated acid and about 50 percent of the monosulfonated acid. All of the baths produced bright ductile plates on polished steel.

The following is an example of a nickel sulfamate plating bath:

The following is an example of a plating bath with chlorocoumarin nickel sulfonate (believed to contain

TABLE 2

| Bath constituent                                                   | I                           | II                          | III                         | IV                          | V                           |
|--------------------------------------------------------------------|-----------------------------|-----------------------------|-----------------------------|-----------------------------|-----------------------------|
| Nickel sulfate, $\text{NiSO}_4 \cdot 6\text{H}_2\text{O}$ , g./l.  | 360                         | 360                         | 360                         | 360                         | 360                         |
| Nickel chloride, $\text{NiCl}_2 \cdot 6\text{H}_2\text{O}$ , g./l. | 30                          | 30                          | 30                          | 30                          | 30                          |
| Boric acid, $\text{H}_3\text{BO}_3$ , g./l.                        | 42                          | 42                          | 42                          | 42                          | 42                          |
| Sulfonated coumarin product, g./l.                                 | 9.7                         | 7.3                         | 11.4                        | 15.5                        | 18.7                        |
| Ferrous sulfate, $\text{FeSO}_4 \cdot 7\text{H}_2\text{O}$         | 14.5                        | 13.0                        | 13.5                        | 12.5                        | 12.5                        |
| Equivalent iron concentration, g./l.                               | 2.9                         | 2.6                         | 2.7                         | 2.5                         | 2.5                         |
| Zinc sulfate, $\text{ZnSO}_4 \cdot 7\text{H}_2\text{O}$ , g./l.    | 1.1                         | 0.9                         | 1.1                         | 0.5                         | 0.45                        |
| Equivalent zinc concentration, g./l.                               | 0.25                        | 0.20                        | 0.25                        | 0.12                        | 0.10                        |
| Wetting agent solution (XXXD), percent by volume                   | 1.0                         | 1.0                         | 1.0                         | 1.0                         | 1.0                         |
| pH                                                                 | 3.1 to 3.9                  | 3.1 to 3.9                  | 2.1 to 2.7                  | 3.1 to 3.6                  | 3.1 to 3.6                  |
| Operating condition:                                               |                             |                             |                             |                             |                             |
| Temperature, °F                                                    | 130 to 133                  | 130 to 133                  | 130 to 133                  | 145                         | 145                         |
| Cathode current density, amp./sq. ft.                              | 30 to 40                    | 30 to 40                    | 45 to 50                    | 57                          | 57                          |
| Agitation (horizontal paddles moving up and down)                  | 60-C. P. M., 4½-inch stroke | 60-C. P. M., 4½-inch stroke | 60-C. P. M., 4½-inch stroke | 60-C. P. M., 4½-inch stroke | 60-C. P. M., 4½-inch stroke |
| Plating time, minutes                                              | 60                          | 60                          | 45                          | 30                          | 30                          |
| Thickness of plate, inch                                           | 0.0015                      | 0.0015                      | 0.0015                      | 0.0015                      | 0.0015                      |
| Surface roughness (profilometer) measurements:                     |                             |                             |                             |                             |                             |
| Before plating, R. M. S. micro-inches                              | 11 to 16                    | 8 to 17                     | 13 to 19                    | 11 to 13                    | 14 to 19                    |
| After plating, R. M. S. micro-inches                               | 1½ to 3                     | 3 to 5                      | 2 to 3                      | 3 to 4                      | 4 to 5                      |
| Plate composition                                                  | Not determined              | 83% Ni, 14% Fe, 3% Zn       | 82% Ni, 14.4% Fe, 3.7% Zn   | Not determined              | Not determined              |

TABLE 3

| Bath constituent                                                                                                  | VI                                        | VII                            | VIII                                            | IX                                   |
|-------------------------------------------------------------------------------------------------------------------|-------------------------------------------|--------------------------------|-------------------------------------------------|--------------------------------------|
| Nickel sulfate, $\text{NiSO}_4 \cdot 6\text{H}_2\text{O}$ , g./l.                                                 | 360                                       | 360                            | 360                                             | 360                                  |
| Nickel chloride, $\text{NiCl}_2 \cdot 6\text{H}_2\text{O}$ , g./l.                                                | 30                                        | 75                             | 75                                              | 75                                   |
| Boric acid, $\text{H}_3\text{BO}_3$ , g./l.                                                                       | 42                                        | 40                             | 42                                              | 42                                   |
| Nickel coumarin sulfonate, the sulfonated portion of which contained 50% disulfonate and 50% monosulfonate, g./l. | 6                                         | 6                              | 6                                               | 7.1                                  |
| Ferrous sulfate, $\text{FeSO}_4 \cdot 7\text{H}_2\text{O}$ , g./l.                                                | 10.0                                      | 10.0                           | 9.5                                             | 4.5                                  |
| Equivalent iron concentration, g./l.                                                                              | 2.0                                       | 2.0                            | 1.9                                             | 0.9                                  |
| Zinc sulfate, $\text{ZnSO}_4 \cdot 7\text{H}_2\text{O}$ , g./l.                                                   | 0.6                                       | 0.5                            | 0.75                                            | 0.7                                  |
| Equivalent zinc concentration, g./l.                                                                              | 0.13                                      | 0.11                           | 0.17                                            | 0.15                                 |
| Wetting agent solution                                                                                            | About 1%, by volume 3.1 to 3.4            | About 1%, by volume 3.0 to 3.2 | About 1%, by volume 3.3                         | About 1%, by volume 3.2              |
| Operating condition:                                                                                              |                                           |                                |                                                 |                                      |
| Temperature, °F                                                                                                   | 135 to 140                                | 115 to 120                     | 137                                             | 135 to 140                           |
| Cathode current density, amp./sq. ft.                                                                             | 50 to 60                                  | 60 to 70                       | 40 to 42                                        | 50 to 60                             |
| Agitation                                                                                                         | Work bar: 35 C. P. M., 6-inch stroke      | Mechanical stirring            | Tumbled in Lucite barrel rotating at 5 C. P. M. | Work bar: 45 C. P. M., 4-inch stroke |
| Plating time, minutes                                                                                             | 20                                        | 4 to 5                         | 30                                              | 5                                    |
| Thickness of plate, inch                                                                                          | 0.001                                     | 0.0002                         | 0.001                                           | 0.0002                               |
| Basis metal                                                                                                       | Polished steel                            | Pickled copper                 | Steel shot                                      | Copper-plated zinc die coatings      |
| Appearance of plate                                                                                               | Mirrorlike—no polishing scratches evident | Mirrorlike, smooth             | Bright and smooth                               | Mirrorlike, smooth                   |
| Approximate composition of plate                                                                                  | 90% Ni, 9% Fe, 1% Zn                      | 90% Ni, 9% Fe, 1% Zn           | Not determined                                  | Not determined                       |

## Example X

|                                                                            |                    |      |
|----------------------------------------------------------------------------|--------------------|------|
| Nickel sulfamate, $\text{Ni}(\text{H}_2\text{NSO}_3)_2$                    | g./l.              | 450  |
| Boric acid, $\text{H}_3\text{BO}_3$                                        | g./l.              | 30   |
| Wetting agent solution                                                     | g./l.              | 0.85 |
| Nickel coumarin sulfonate containing about 40% nickel coumarin disulfonate | g./l.              | 5    |
| Zinc sulfate, $\text{ZnSO}_4 \cdot 7\text{H}_2\text{O}$                    | g./l.              | 0.5  |
| Equivalent zinc concentration                                              | g./l.              | 0.11 |
| Ferrous sulfate, $\text{FeSO}_4 \cdot 7\text{H}_2\text{O}$                 | g./l.              | 5    |
| Equivalent iron concentration                                              | g./l.              | 1    |
| pH                                                                         |                    | 2.7  |
| Operating conditions:                                                      |                    |      |
| Cathode current density                                                    | 50 amp./sq. ft.    |      |
| Temperature                                                                | 125 to 135° F.     | 70   |
| Agitation                                                                  | Mechanical stirrer |      |
| Plating time                                                               | 25 minutes         |      |

Bright plate and leveling of surface irregularities were obtained with the above conditions. Plate composition was not determined.

## about 50 percent nickel monochloro, disulfono coumarin):

## Example XI

|                                                            |                   |      |
|------------------------------------------------------------|-------------------|------|
| Nickel sulfate, $\text{NiSO}_4 \cdot 6\text{H}_2\text{O}$  | g./l.             | 300  |
| Nickel chloride, $\text{NiCl}_2 \cdot 6\text{H}_2\text{O}$ | g./l.             | 30   |
| Boric acid, $\text{H}_3\text{BO}_3$                        | g./l.             | 41   |
| Ferrous sulfate, $\text{FeSO}_4 \cdot 7\text{H}_2\text{O}$ | g./l.             | 10.0 |
| Equivalent iron concentration                              | g./l.             | 2.0  |
| Zinc sulfate, $\text{ZnSO}_4 \cdot 7\text{H}_2\text{O}$    | g./l.             | 0.5  |
| Equivalent zinc concentration                              | g./l.             | 0.11 |
| Wetting agent solution (XXXD)                              | percent by volume | 1.0  |

pH 2.9 to 3.5  
Nickel chlorocoumarin sulfonate g./l. 6

Using a work-bar agitating at 53 C. P. M. with a 3½-inch stroke, leveling was measured at different current densities and temperatures, with the results shown in Table 4. All plates were mirrorlike and ductile. Plate composition was not determined.

## Example XII

Exceptionally good plates were obtained with iron and zinc using a plating bath prepared as follows:

TABLE 4

## EFFECT OF CHLOROCOUMARIN NICKEL SULFONATE ON LEVELING AT VARIOUS OPERATING CONDITIONS

| Zinc in bath, g./l. | Temp.,<br>°F. | Current<br>density,<br>amp./<br>sq. ft. | Leveling,<br>percent |
|---------------------|---------------|-----------------------------------------|----------------------|
| 0.1                 | 135           | 30                                      | 28                   |
| 0.1                 | 135           | 30                                      | 34                   |
| 0.1                 | 135           | 50                                      | 27                   |
| 0.1                 | 135           | 70                                      | 34                   |
| 0.1                 | 160           | 30                                      | 17                   |
| 0.1                 | 160           | 50                                      | 24                   |
| 0.1                 | 160           | 70                                      | 22                   |
| 0.1                 | 160           | 70                                      | 18                   |
| 0.2                 | 135           | 30                                      | 40                   |
| 0.2                 | 135           | 50                                      | 34                   |
| 0.2                 | 135           | 50                                      | 47                   |
| 0.2                 | 135           | 70                                      | 40                   |
| 0.2                 | 135           | 70                                      | 42                   |
| 0.2                 | 160           | 30                                      | 35                   |
| 0.2                 | 160           | 50                                      | 45                   |
| 0.2                 | 160           | 70                                      | 46                   |

NOTE.—Thickness of all plates equal to 0.001 inch.  
percent leveling =  $100(B-A)$

B

where B=R. M. S. profilometer reading in microinches before plating  
A=R. M. S. profilometer reading in microinches after plating

| Components:                                                               | Amount                |
|---------------------------------------------------------------------------|-----------------------|
| Nickel sulfate ( $\text{NiSO}_4 \cdot 6\text{H}_2\text{O}$ )              | g./l. 360             |
| Nickel chloride ( $\text{NiCl}_2 \cdot 6\text{H}_2\text{O}$ )             | g./l. 30              |
| Iron sulfate ( $\text{FeSO}_4 \cdot 6\text{H}_2\text{O}$ )                | g./l. 15              |
| Equivalent iron concentration                                             | g./l. 3.0             |
| Zinc sulfate ( $\text{ZnSO}_4 \cdot 7\text{H}_2\text{O}$ )                | g./l. 0.7             |
| Equivalent zinc concentration                                             | g./l. 0.15            |
| Boric acid ( $\text{H}_3\text{BO}_3$ )                                    | g./l. 42              |
| Sulfonation product of one part coumarin and 5 parts fuming sulfuric acid | g./l. 12.9            |
| "XXXD"                                                                    | percent by volume 0.5 |
| Water                                                                     | Balance               |

With a temperature of 136° F., a pH of 3.8, an anode current density of 20 amp./sq. ft., a cathode current density of 30 amp./sq. ft. and with the solution agitated with Bakelite paddles reciprocating about 54 C. P. M. with a 4-inch stroke, a uniformly mirrorlike plate, 0.00095-inch thick measuring 2.5 R. M. S. microinches was obtained on a steel bumper-bar segment measuring 11 R. M. S. microinches before plating. The plate contained approximately 3 percent iron and 3 percent zinc.

A plating bath using sulfonated 1,4-benzopyrone or chromone was formulated as follows:

## Example XIII

| Components:                                                              | Amount              |
|--------------------------------------------------------------------------|---------------------|
| Nickel sulfate ( $\text{NiSO}_4 \cdot 6\text{H}_2\text{O}$ )             | g./l. 360           |
| Nickel chloride ( $\text{NiCl}_2 \cdot 6\text{H}_2\text{O}$ )            | g./l. 30            |
| Boric acid ( $\text{H}_3\text{BO}_3$ )                                   | g./l. 42            |
| Iron sulfate ( $\text{FeSO}_4 \cdot 7\text{H}_2\text{O}$ )               | g./l. 5.5           |
| Equivalent iron concentration                                            | g./l. 1.1           |
| Zinc sulfate ( $\text{ZnSO}_4$ )                                         | g./l. 1.25          |
| Equivalent zinc concentration                                            | g./l. 0.5           |
| Product of sulfonating 1 part chromone with 5 parts fuming sulfuric acid | g./l. 18            |
| "XXXD"                                                                   | percent by volume 1 |
| Water                                                                    | Balance             |

10  
The pH of the bath was adjusted to 2.9 and the temperature thereof was maintained at about 130° F. With the anode at a current density of 10 amp./sq. ft. and the cathode at a current density of 20 amp./sq. ft. and being moved with a 3-inch stroke at 60 C. P. M., a nearly mirror-bright, very ductile nickel plate 0.0015-inch measuring 6 R. M. S. microinches over steel measuring 9 R. M. S. microinches was produced.

The invention is not limited to the preferred embodiment but may be otherwise embodied or practiced within the scope of the following claims.

We claim:

1. A bath for depositing a nickel alloy electroplate, comprising an acidic aqueous solution of about 17 to 233 g./l. of nickel ions, about 0.3 to 5.6 g./l. of iron ions, about 0.03 to 1.25 g./l. of zinc ions, and a disulfonated benzopyrone in an amount equivalent to about 1 to 10 g./l. of coumarin disulfonic acid.
2. A bath for depositing a nickel alloy electroplate, comprising an acidic aqueous solution of about 34 to 120 g./l. of nickel ions, about 0.5 to 3.0 g./l. of iron ions, about 0.03 to 0.20 g./l. of zinc ions, and a disulfonated benzopyrone in an amount equivalent to about 1 to 10 g./l. of coumarin disulfonic acid.
3. A bath for depositing a nickel alloy electroplate, comprising an acidic aqueous solution of about 17 to 233 g./l. of nickel ions, about 0.3 to 5.6 g./l. of iron ions, about 0.03 to 1.25 g./l. of zinc ions, and a sulfonated benzopyrone product, the sulfonated portion of which contains at least about 50 percent by weight of disulfonated benzopyrone, said sulfonated benzopyrone product being present in an amount equivalent to about 1 to 10 g./l. of coumarin disulfonic acid.
4. A bath for depositing a nickel alloy electroplate, comprising an acidic aqueous solution of about 34 to 120 g./l. of nickel ions, about 0.5 to 3.0 g./l. of iron ions, about 0.03 to 0.20 g./l. of zinc ions, and a sulfonated benzopyrone product, the sulfonated portion of which contains at least about 50 percent by weight of disulfonated benzopyrone, said sulfonated benzopyrone product being present in an amount equivalent to about 1 to 10 g./l. of coumarin disulfonic acid.
5. In a process of depositing a nickel alloy electroplate, the step of passing an electric current through an electrolyte between an anode and a cathode, said electrolyte comprising an acidic aqueous solution of about 17 to 233 g./l. of nickel ions, about 0.3 to 5.6 g./l. of iron ions, about 0.03 to 1.25 g./l. of zinc ions, and a disulfonated benzopyrone in an amount equivalent to about 1 to 10 g./l. of coumarin disulfonic acid.
6. In a process of depositing a nickel alloy electroplate, the step of passing an electric current through an electrolyte between an anode and a cathode, said electrolyte comprising an acidic aqueous solution of about 34 to 120 g./l. of nickel ions, about 0.5 to 3.0 g./l. of iron ions, about 0.03 to 0.20 g./l. of zinc ions, and a disulfonated benzopyrone in an amount equivalent to about 1 to 10 g./l. of coumarin disulfonic acid.
7. In a process of depositing a nickel alloy electroplate, the step of passing an electric current through an electrolyte between an anode and a cathode, said electrolyte comprising an acidic aqueous solution of about 17 to 233 g./l. of nickel ions, about 0.3 to 5.6 g./l. of iron ions, about 0.03 to 1.25 g./l. of zinc ions, and a sulfonated benzopyrone product, the sulfonated portion of which contains at least about 50 percent by weight of disulfonated benzopyrone, said sulfonated benzopyrone product being present in an amount equivalent to about 1 to 10 g./l. of coumarin disulfonic acid.
8. In a process of depositing a nickel alloy electroplate, the step of passing an electric current through an electrolyte between an anode and a cathode, said electrolyte comprising an acidic aqueous solution of about 34 to 120 g./l. of nickel ions, about 0.5 to 3.0 g./l. of iron ions, about 0.03 to 0.20 g./l. of zinc ions, and a sulfonated benzopyrone product, the sulfonated portion of which contains at least about 50 percent by weight of disulfonated benzopyrone, said sulfonated benzopyrone product being present in an amount equivalent to about 1 to 10 g./l. of coumarin disulfonic acid.

11

g./l. of nickel ions, about 0.5 to 3.0 g./l. of iron ions, about 0.03 to 0.20 g./l. of zinc ions, and a sulfonated benzopyrone product, the sulfonated portion of which contains at least about 50 percent by weight of disulfonated benzopyrone, said sulfonated benzopyrone product being present in an amount equivalent to about 1 to 10 g./l. of coumarin disulfonic acid.

5

12

References Cited in the file of this patent

## UNITED STATES PATENTS

|           |              |               |
|-----------|--------------|---------------|
| 1,837,355 | Burns et al. | Dec. 22, 1931 |
| 1,960,029 | Russell      | May 22, 1934  |
| 2,418,970 | Donroe       | Apr. 15, 1947 |
| 2,513,280 | Brown        | July 4, 1950  |
| 2,694,041 | Brown        | Nov. 9, 1954  |
| 2,809,156 | Safranek     | Oct. 8, 1957  |